

Oct. 5, 1943.

J. W. WRIGHT

2,330,940

FIRE EXTINGUISHER

Filed Jan. 18, 1940

2 Sheets-Sheet 1



Inventor

John W Wright  
Marshall & Nee

Attorneys

Oct. 5, 1943.

J. W. WRIGHT

2,330,940

FIRE EXTINGUISHER

Filed Jan. 18, 1940

2 Sheets-Sheet 2



Fig. 2



Fig. 5

Fig. 6



Fig. 4

Fig. 8

## UNITED STATES PATENT OFFICE

2,330,940

## FIRE EXTINGUISHER

John W. Wright, Dayton, Ohio, assignor to The Fyr-Fyter Company, Dayton, Ohio, a corporation of Ohio

Application January 18, 1940, Serial No. 314,425

3 Claims. (Cl. 220—64)

This invention relates to fire extinguishers.

It is the principal object of the invention to provide a fire extinguisher that is light in weight, relatively strong in construction and capable of withstanding normal usage, inexpensive to manufacture, and which will resist rupture and leakage at the seams under the application of high pressure over long periods of use, and under repeated applications of such pressure.

A further object is the provision of a welded fire extinguisher casing of this character which is light in weight, easy to manipulate, and is fabricated from sheet metal having high strength providing a welded construction free of rivets, and having no solder, brazing materials, or the like.

It is a further object to provide such a fire extinguisher in which the interior of the casing is effectively protected against the corrosive action of chemicals by means of a thin, uniform protective coating overlying the entire interior thereof.

It is a still further object to provide such an extinguisher in which such coating is applied economically and uniformly by electroplating to form an electrolytically deposited protective coating thereon.

It is a still further object to provide a simple and satisfactory process for the economical manufacture of fire extinguisher casings of the above character.

Other objects and advantages will be apparent from the following description, the accompanying drawings, and the appended claims.

In the drawings—

Fig. 1 is a view in elevation of a finished extinguisher casing constructed in accordance with the present invention and showing in dotted outline the electroplating anode in position for forming the inner protective coating;

Fig. 2 is a partial view in section of the upper end of the casing showing the manner of securing the upper dome or closure member in position on the body shell;

Fig. 3 is a sectional view showing the manner of securing the bottom closure member in position;

Fig. 4 is a detail view in perspective showing a preliminary step in the forming operation in which the body shell is rolled into cylindrical form of predetermined diameter and temporarily secured;

Fig. 5 is a broken perspective view showing the manner in which the longitudinal seam is welded;

Fig. 6 is a diagrammatic view showing the welding operations and the controls therefor;

Fig. 7 is a sectional view through the welded joint on an enlarged scale; and

Fig. 8 is a view showing a modified procedure for securing the bottom closure member in place.

Casings for fire extinguishers of the customary portable or manually operable type in commercial use at the present time are usually fabricated from sheet copper and are of riveted and soldered construction. While copper possesses desirable corrosion-resisting properties, it is not a particularly strong material and relatively heavier sections must be used to secure the required strength for an extinguisher casing. Where a riveted seam is used, it has been found necessary to solder over the head of each rivet and around the edges of the seam in order to assure a tight construction, and this operation has required considerable time and the use of a substantial quantity of solder. Solder has likewise been applied over the entire interior of the casing to protect against corrosion under the action of the chemicals forming the charge, and this operation further adds to the expense of manufacture and to the weight, particularly as it is difficult to secure a uniform application of the solder and an excess is usually applied. Further the physical properties of the copper shell are such that if heated materially above the proper temperature for the application of the solder, definite impairment of its physical properties results, and consequently considerable care is necessary in the manufacture of such extinguisher casings. Such fire extinguishers are customarily made in two and one-half gallon size, and the construction as above described results in an extinguisher casing having substantial weight, making shipment more expensive and manipulation and use more difficult.

In accordance with the present invention a material is utilized for the formation of the shell which has higher strength than the copper heretofore used and which will withstand equal or even greater pressure in a section of reduced thickness. Thus very satisfactory results have been secured from the use of such material in an extinguisher shell with a reduction in weight of approximately 25%, resulting not only in more economic use of materials, but reducing transportation and packaging costs and facilitating the handling of the extinguisher in actual use.

Further the invention provides for the forming and the fabrication of the shell and the finished casing in such a manner as to completely dispense with the necessity for riveting and soldering at the seams. This results in further economies in manufacture and provides a finished shell

which is less likely to result in failure by reason of decomposition taking place in the area of the seams. In order to provide the desired resistance to corrosion under the action of the chemicals which are contained within the casing, a thin and substantially uniform protective surface is formed over the entire interior in place of the previous practice of applying a surface by tinning or soldering.

In accordance with this invention the added weight and expense of a coating of solder are eliminated and a uniform highly effective coating is formed upon the interior surface by electrolytic deposition. Such operation provides for securing a uniform application of the coating, over the entire interior surface of the casing including the welded seam areas, to a proper depth to afford protection against failure, and avoiding unnecessary waste of material. The coating preferably comprises a plating of nickel which is electrolytically formed from a suitable nickel solution. Since the seams of the casing are free of rivets and there is no solder or the like, the interior of the casing presents only the surface of the metal thereof and hence may be uniformly plated with a uniform, long lasting protective coating which will not be readily subject to decomposition. A highly satisfactory coating, capable of adequately withstanding the presence of the customary fire extinguisher chemicals over long periods of time is thus provided.

Referring to the drawings which disclose a preferred embodiment of the invention, the fire extinguisher casing is shown generally at 10. It comprises a main cylindrical body portion or shell 11, an upper closure or dome member 12, and a bottom closure member 13. The upper dome member is formed with a filling opening 14, the neck 15 defining such opening having an exterior threaded portion 16 for removably receiving a cap thereon. The dome also contains a discharge fitting 17 passing through the wall thereof and having a screen 18 upon its inner surface and a connection shown at 19 for receiving flexible hose carrying a discharge nozzle, in the usual manner. The closure member 13 is preferably located somewhat above the lower end of the body shell 11, and above an inwardly recessed flange 20, to provide a space for a handle 21. A supporting bead 22 is formed at the bottom rim upon which the extinguisher may be supported in standing position. It will also be understood that suitable hand brackets may be positioned upon the dome, and likewise a nameplate may be fastened to the surface of the extinguisher.

In accordance with the present invention a flat sheet of metal is rolled into the generally cylindrical form of the shell 11 and received within one or more gage members 25. Such gage member has an internal diameter corresponding to the desired external diameter of the shell, and the two ends of the cylindrical shell are lapped upon each other to provide the overlapping joint as shown at 26, one edge of the shell material preferably being offset as shown at 27 in order to form a more uniform exterior surface upon the finished extinguisher. With the shell in such position it is temporarily tacked in place at the overlapping joint by suitable means such as by spot welding electrodes indicated at 30. These electrodes may be moved along the longitudinal joint, one outside and one inside the cylinder, and several spot welds made along the length of

the shell, sufficient in number to securely hold the same in the proper rolled or formed position. Usually about four such spot welding applications are found entirely sufficient. It will be noted that in this operation the metal sheet is brought in surface to surface contact with itself, and that there is no intermediate use of solder or other similar auxiliary material.

The cylinder is then subjected to a welding operation to securely weld the longitudinal overlapping joint along its entire length. In order to effectively secure such joint so that it will withstand the necessary high pressure conditions to which it is subjected in use it is important that it be secured at a number of closely spaced points along its length. It is also important however that the welding operations be so carried out as to avoid developing an excessive heat throughout the welded area or in the metal immediately adjacent thereto, such as might result in weakening the physical characteristics of the shell material with the accompanying possibility of failure. The material which applicant prefers to utilize for the manufacture of the shell comprises a metal which has reasonably satisfactory inherent resistance to decomposition, high strength, and also the ability to be electrically welded, that is, possessing suitable characteristics of electrical resistance. A preferred material for this purpose consists of a copper-silicon alloy, containing primarily copper and silicon, the silicon comprising not more than 3.5% of the material, and to which may be also added small quantities of one or more alloying elements, such, for instance, as zinc, tin, or manganese, the total quantity of these alloying elements being less than 2.0% of the entire material. One alloy which has been successfully used for this purpose consists of copper, 96.25%; silicon, 3.25% and tin, 0.50%. Another alloy which has been successfully used consists of copper, 97.75%; silicon, 2.00% and tin, 0.25%.

While such alloy has the desired high tensile strength, of the order of 85,000 pounds per square inch, it cannot be heated to a high temperature without serious injury to such properties and marked reduction in such tensile strength. Accordingly therefore means are provided for producing a welding operation in spaced areas along the lapped joint, sufficiently close to provide for securely sealing the joint upon itself and preventing any rupture or leakage thereof in use, and so spaced that the heat generated during the welding operation is not sufficiently great in the immediate vicinity of the weld as to result in damage to the physical properties of the metal.

For this purpose the cylindrical body is moved relative to inner and outer welding electrodes, and the welding operation is controlled in an intermittent manner during such relative movement. That is, the welding current is supplied intermittently to such electrodes, thereby providing welded areas alternating with non-welded areas. By suitably controlling the rate of such relative travel, and the frequency and duration of the periods of such current supply and non-supply, proper regulation and spacing of the welded areas may be secured as desired. This results in producing seams in the welded areas, which may be as closely spaced as necessary to provide for adequately securing the overlapping parts together, and at the same time sufficiently separated to avoid development of such excessive quantities of heat as to impair the properties of the metal. Simultaneously the parts are

subjected to substantial pressure, so that during the entire feeding operation including both periods of welding and non-welding, the overlapping edges are firmly pressed into surface to surface contact.

This is shown diagrammatically in Fig. 6 where the cylinder 11 is being moved relative to the inner and outer electrodes 35, 36, which are supplied with flow of welding current from the secondary of a step-down transformer 37. The primary is energized from a suitable power source of alternating current (not shown), through a control indicated diagrammatically at 40. Such control is of the electronic control type using for example ignitron or thyratron tubes, providing for selection of the length of time during which the transformer is energized, and the corresponding independent control of the length of time during which it is not energized. By suitably regulating the control, the transformer may be energized and current caused to flow in the welding circuit for any desired period of time from a half cycle up, and this may be followed by a period of non-flow of welding current likewise variable from a half cycle up. With continuous movement of the electrodes relative to the cylindrical body it will thus be clear that seams or stitches may be formed in the metal of any desired width and spacing with respect to each other. An adjustable tap 41 on the transformer provides for adjusting the voltage and hence the amount of flow of the welding current. Also means are provided as shown at 42 in the form of an air cylinder for exerting pressure upon the electrodes and through them upon the parts being welded.

As a specific example of conditions which have been found to produce highly satisfactory results in actual operations, a welding current of the order of 20,000 amperes has been used with a rate of travel of the cylinder relative to the electrodes of 36 inches per minute. Using a current of a frequency of 60 cycles per second, and with the control 40 set to provide welding current for three cycles followed by a like period of non-welding, this will result in a welded seam comprising a welded area of .03 inch in length followed by a space of .03 inch which is not welded. During these operations the welding electrodes are pressed toward each other with a total force of approximately 700 pounds by means of air cylinder 42. As shown in Fig. 7 these welded areas 43 alternate with non-welded areas 44, producing the effect of seams or stitches in the metal, adequate to securely hold the welded parts together and yet so spaced from each other that the entire body of the metal in the vicinity of the weld is not highly heated during the operation such as to cause loss of its physical properties. A firm and permanent joint having even greater strength than the main body of the shell is thus secured.

Having completely welded the longitudinal overlapping joint, the end closure members which have been previously fabricated, preferably from the same metal alloy as described above and in the usual manner, are then fastened to the shell. It is preferred to subject these parts, after fabrication, to a stress-relieving heat treatment to relieve strain induced in the material by the forming operations. Such stress-relieving heat treatment may vary somewhat for different alloys used to fabricate these parts, but in using the alloy described above, such parts may be heated to a temperature of 550° F. to 600° F., maintained at this temperature for a period of one-half hour, 75

and then quenched in water. This is preferably accomplished by first fastening the dome 12 in position upon one end of the shell 11. The dome is provided with an outwardly extending flange 45 which is telescopically received over the end of the shell, and a pair of welding electrodes comprising an internal wheel 46 and an external wheel 47 are brought into cooperative relation with respect to such flanged portion. Inner wheel 46 may be relatively large in diameter and supported from an arm extending through the open bottom end of the shell, the shell and the dome being preferably rotated around their longitudinal axis between the welding electrodes 46, 47. Such rotation may be effected by any suitable means, as, for instance, by causing the outer electrode 47 to be positively rotated by means of gear-wheels 48 and 49. Current is supplied to such electrodes in the same intermittent and controlled manner as above described with respect to the longitudinal seam, to secure such end closure member in place upon the shell in a similar effective manner, without the use of solder or rivets, and producing the stitch form of the final welded joint.

Thereafter the bottom closure member 13 is slipped into position over the bead 20, formed in the shell by rolling, the shell being slightly flattened to permit its introduction. Such member is likewise welded in place through the use of welding electrodes consisting of inner roller 50 and outer roller 51 cooperating with each other under pressure in the manner above described. Roller 50 is made small enough to be passed through the filling opening 14, and is supported upon a suitable arm extending through such opening.

After the bottom closure is in position the casing is completely fabricated and presents a smooth and pleasing finished appearance showing the presence of the longitudinal seam 55 and the peripheral seams 56 and 57 upon its outer surface.

In order to form the inner protective coating 45 upon the surface of the extinguisher to protect the same against the highly corrosive chemicals which are used, an electrolytic deposit of non-corrosive metal is made throughout the entire interior surface of the extinguisher. This is effected by filling the casing with a suitable electroplating solution, inserting an anode shown at 60 in dotted lines into the solution, and making suitable electrical connection to such anode and to the casing itself which forms a cathode, and supplying direct current thereto.

The coating which has been found to produce highly satisfactory results is a nickel coating. The anode is preferably formed of substantially pure nickel and is suspended in a solution containing 64 grams per liter of metallic nickel in the form of nickel chloride and nickel sulfate. As an example of satisfactory plating conditions, direct current of approximately 100 amperes is passed through the solution for a period of about an hour. The passage of the current results in a rise of temperature of the solution and a change in the electrical resistance so that preferably the current flow is controlled by suitable regulating devices so that its value is maintained substantially constant. Likewise it is desirable to enclose the anode in a suitable bag or container of glass cloth or the like to prevent the settlement of sludge and foreign particles from the anode which would otherwise be deposited upon the bottom of the extinguisher.

Such electroplating operation provides for forming a substantially uniform coating having such thickness as to afford the proper protection against failure in use. It is found that it should not be less than about .0006 inch thick all over and to assure a satisfactory thickness of coating with some margin of safety it is preferred to make it approximately .001 inch thick. Being substantially uniformly deposited over the entire interior of the extinguisher including the welded areas, the joints and seams, a thoroughly effective protection is thereby secured and without waste or unnecessary thickness of material at any point. It adds about 2 oz. in weight to the extinguisher and affords substantially better protection against corrosion than the former use of a tin lead alloy applied by a tinning operation at the seams, over rivets, and the entire inner surface, which would usually add in the range of 2 to 4 pounds in extra weight.

Following the plating operation the exterior surface of the shell may be finished in customary manner such as by polishing, enamel coating and the like and the extinguisher is then in form so that it is suitable for use.

Fig. 8 shows a somewhat modified form of construction in which the necessity for welding the bottom closure member 13 in place by means of an arm passing through the filling opening is avoided. In this arrangement a closure member 63 is positioned within the cylindrical body 60 with its convex face inwardly after which welding wheels 64 and 65 may be brought into cooperative relation with respect to the flanged portion, both such wheels being of suitable size and capable of being firmly supported and pressed towards each other under suitable pressure. Similar intermittent control during relative movement of the electrodes with respect to the parts to be welded is provided, so that an effectively sealed welded joint is provided in the manner above described. After welding, the projecting edge 61 of cylindrical body 60 may be turned inwardly as indicated at 62 forming a flanged portion serving as a base or support for the extinguisher to rest upon when the device is in the upright position and presenting a smooth rounded edge to prevent injury during operation. A suitable handle 66 may be affixed to the bottom of the shell as indicated in Fig. 8 by suitable means such, for instance, as by means of spot-welding the handle 66 to the inwardly turned flange 62.

While the processes and articles herein described constitute preferred embodiments of the invention, it is to be understood that the invention is not limited to these precise processes and articles, and that changes may be made therein without departing from the scope of the invention which is defined in the appended claims.

What is claimed is:

1. A fire extinguisher of the character described comprising a substantially cylindrical tubular casing member formed from a sheet of copper silicon alloy having high strength and adapted to be electrically welded and having portions of said metal sheet overlapping along a longitudinal edge, said overlapping portions of

said metal sheet being in surface to surface contact in the cylindrical surface and electrically welded directly to each other along the length of said seam, a dome member on said casing extending in one direction and having a flange portion thereof extending in the opposite direction and received in overlapping relation on one end of said tubular casing member, a bottom closure member on said casing and also extending in one direction with a flange portion thereof extending in the opposite direction thereto and received on the other end of said tubular casing member, the flanges of said dome and said bottom closure members being electrically welded directly to the metal surface of said tubular casing member around the entire periphery thereof, each of the welds along said longitudinal joint and around the periphery of said closure members comprising a series of separated welded areas each of predetermined size and in such number as to provide for effectively sealing the joint and being so spaced as to avoid excessive heating of the body of the metal sheet outside of said welded areas, said casing member having a protective coating upon the entire inner surface thereof including the welded areas of a character adapted to resist corrosion from the contents of the extinguisher.

2. A fire extinguisher of the character described comprising a substantially cylindrical tubular casing member formed from copper silicon alloy of high strength and adapted to be electrically welded and having portions of said metal sheet overlapping along a longitudinal edge, said overlapping portions of said metal sheet being in surface to surface contact in the cylindrical surface and electrically welded directly to each other along the length of said seam, a dome member on said casing extending in one direction and having a flange portion thereof, extending in the opposite direction and received in overlapping relation on one end of said tubular member, a bottom closure member on said casing and also extending in one direction with a flange portion thereof extending in the opposite direction thereto and received on the other end of said tubular member, the flanges of said dome and said bottom closure members being electrically welded directly to the metal surface of said tubular member around the entire periphery thereof providing a smooth interior surface adapted for plating, each of the welds along said longitudinal joint and around the periphery of said closure members comprising a series of separated welded areas each of predetermined size and in such number as to provide for effectively sealing the joint and being so spaced as to avoid excessive heating of the body of the metal sheet outside of said welded areas, and the entire inner surface of said extinguisher casing including the welded areas having a plating of nickel electrolytically applied in substantially uniform manner thereto.

3. A fire extinguisher as defined in claim 2 in which the electrodeposited plating of nickel has a thickness not less than approximately .0006 inch.

JOHN W. WRIGHT.